

Dec. 26, 1961

C. H. BOMMERSCHEIM

3,014,851

PROCESS FOR PLATING A SELECTIVE SURFACE WITHIN A GROOVE

Filed June 5, 1959

2 Sheets-Sheet 1



*Fig. 1.*



*Fig. 2.*

INVENTOR.  
CHARLES HENRY BOMMERSCHEIM

BY  
*Max R. Millman*

ATTORNEY.

Dec. 26, 1961

C. H. BOMMERSCHEIM

3,014,851

PROCESS FOR PLATING A SELECTIVE SURFACE WITHIN A GROOVE

Filed June 5, 1959

2 Sheets-Sheet 2

Fig. 3.



Fig. 4.



Fig. 5.



INVENTOR.  
CHARLES HENRY BOMMERSCHEIM

BY  
May R. Millman

ATTORNEY.

1

3,014,851

PROCESS FOR PLATING A SELECTIVE SURFACE  
WITHIN A GROOVE

Charles Henry Bommersheim, Kalamazoo, Mich., assignor to Savage Plating &amp; Anodizing Co., Inc., Kalamazoo, Mich., a corporation of Michigan

Filed June 5, 1959, Ser. No. 818,287

6 Claims. (Cl. 204—15)

This invention relates to a process and apparatus for the metal plating of a selective surface within a groove which is normally subject to wear and/or corrosion.

The primary object of the invention is to provide an efficient and practical method of plating a selective surface of a dimensionally deep and/or narrow groove in such a manner that the plating is of controlled and uniform thickness across the entire selected surface without requiring regrinding or resurfacing after plating.

It is well known that the horizontal land surfaces of cast iron diesel engine and other pistons are subject to wear and/or corrosion. Hence, these land surfaces should be plated with a corrosion and wear resistant metal, such as hard chromium, in thicknesses to meet tolerances.

Heretofore, conventional methods of plating the lands of the ring grooves of pistons have been unsuccessful. For example, when the piston is held in a vertical position and made cathodic and a parallel vertical anode is positioned one to twelve inches therefrom, metal will not deposit on the selected land surface of the ring groove with sufficiently uniform distribution as to coating thickness. Because the groove is dimensionally deep and/or narrow, the deposited metal will build up preferentially at the edge of the surface closest to the anode while the portion at the bottom of the groove which is at the greatest distance from the anode will receive little or no deposit.

If an attempt is made to plate the surfaces within the grooves normally subject to wear and/or corrosion by anodes positioned within the narrow ring grooves, difficulties arise. Thus, if the anodes are lead foil or wire, it is difficult, if not impossible, to support them in such a manner that they are retained at all times in the ring grooves at fixed distances and positions relative to the land surface to be plated. Unless this is done, the deposit will be non-uniform in thickness over the significant surface and too costly to attempt to regrind after plating. Also, if the anode should touch the piston at any point, a short circuit will occur with arcing and injury to the surface and deposit. Moreover, lead wire of sufficient size to carry current would inhibit the entrance of fresh electrolyte and might lead to localized overheating of the electrolyte plus depletion. These considerations also preclude the possibility of supporting and accurately positioning a delicate anode structural shape within a narrow ring groove around the circumference of a piston by means of an outside structure and maintaining accurate spacing between the anode and the surface to be plated.

The present invention overcomes the aforementioned difficulties by using an insoluble anode which is conformable to the contour of the grooved member and which is fixed to but insulated from the grooved member in such a manner that the anode covers the surfaces of the groove not to be plated but opposes the selected surfaces to be plated, the grooved member itself serving to support the anode. By making the grooved member a cathode and immersing the same in a suitable electrolyte, a uniform controlled thickness of such metals as chromium, nickel, copper, tin, zinc, silver, gold or cadmium can be deposited on the selected surfaces of the grooves.

The principles of the invention will best be understood with reference to the accompanying drawings, wherein:

2

FIGURE 1 is an elevational view of apparatus illustrating the present method of plating a selected surface of the ring groove of a piston;

FIGURE 2 is a sectional view taken on the line 2—2 of FIGURE 1;

FIGURE 3 is an enlarged vertical sectional view through a piston illustrating the manner of affixing the insoluble anode to the piston in position to plate a selected surface of the ring groove;

FIGURE 4 is a view similar to FIGURE 3 showing a modified form of the invention; and

FIGURE 5 is a fragmentary diagrammatic view of an alternative method of applying the anode to the piston. Specific reference is now made to the drawings wherein similar reference characters are used for corresponding elements throughout. It should be understood that while the invention will be described with reference to a cast iron diesel engine piston, the principles thereof are applicable to any metallic grooved member where it is necessary or desirable to plate one or more selected surfaces of the groove.

Indicated at 10 is a diesel engine piston which, as is well known, is a cylindrical cast iron member having a plurality of axially spaced ring grooves 12 which are relatively narrow and deep, the depth being approximately 0.25" and the average width approximately 0.253 to 0.255", the overall length of the piston approximating 9.781". When the piston is operated in the engine, the rings in the grooves subject the land surfaces 14 thereof to wear and corrosion which, if not corrected, eventually causes cracking of the rings. Hence, it is desirable that these land surfaces of the new pistons be protected against wear and corrosion by a metal plating, preferably hard chromium. However, the deposited metal must be of controlled and uniform thickness coextensive with the land surface, generally in the order of magnitude of 1 to 2 mils and the present invention accurately and efficiently accomplishes this without the necessity of regrinding or resurfacing of the deposited metal.

A suitable vessel or tank 16 is provided in which is supported a steel rack 18, preferably U-shaped, the rack in turn supporting the piston 10 in a vertical position, the rack including vertically extending insulating members 20. The steel members 22 passing through the insulation include horizontal portions which engage the lower end of the piston 10. Mounted upon a flange or other support on the upper end of the tank are insulators 24 which in turn mount two copper buses 26, the upper ends of the vertical portions of the steel rack members 22 hooking around and contacting the copper buses, the latter being operatively connected to a current source (not shown) which is negative when plating takes place thereby rendering the piston cathodic.

The insoluble anode employed in the process is such as to be conformable to the configuration of the piston and readily affixable but insulated from those portions of the piston which are not to be plated so that the anode is automatically retained by the piston in a desired position adjacent to but opposite the surface or surfaces to be coated. For this purpose an adhesive backed metallic tape is employed. For chromium plating, an adhesive backed insoluble lead tape is preferred, the same being also satisfactory for nickel plating from a chloride-free nickel-sulfate bath or copper plating from a conventional acid copper-sulfate bath. A low carbon steel or alloy steel adhesive backed tape may also be used for plating copper, tin, zinc, silver, gold or cadmium from conventional alkaline electrolytes for these metals. A specific commercially available tape utilizable in the process is pressure sensitive lead tape which consists of a lead foil backed by an adhesive of the type disclosed in U.S. Patent Re. 23,843.

In practice, the land surface 14 to be plated should be given a satisfactory surface finish. In the case of new pistons, the surface finish should be 32 micro inch R.M.S. or better. In the case of worn pistons, the surface finish should be 16 micro inch R.M.S. or better because of the greater thickness of metal deposit which is normally required. The piston is then vapor degreased and an insulating strip 28, such as pressure sensitive tape for electroplating which is disclosed in U.S. Patent Re. 23,843, is applied around the piston to all of those surfaces which are not to be plated, the lower free edge 30 of one strip portion thereof terminating immediately above the land surface 14 to be plated.

The adhesive backed lead tape 32 is then applied to the insulating strip 28 in parallel strips with respect to the piston axis which overlap (shown exaggerated in FIGURE 3) starting approximately half way up the vertical surface 34 of the groove with the land 14 to be plated, as at 36, then across the horizontal surface 38 of the groove opposite the land 14, then up the outside surface 40 of the piston where it terminates at or below the upper transverse surface 42 of the piston as at 44. If necessary, the overlapped strips of lead tape 32 are ultimately smoothed out. A lead wire 46 is then wrapped around the upper portion of the tape 32 gripping the outside of the piston firmly to make positive electrical contact. One or more lead wires 48, see FIGURES 1 and 2, are then carried a sufficient distance above the piston for operative connection to an outside current source whereby the tape is rendered positive during the plating operation.

It is to be understood that the lead tape 32 may be applied to the piston in a series of vertically extending, overlapping strips whose longitudinal axes extend axially of the piston as shown in FIGURE 5 instead of in a series of horizontally extending strips whose axes extend circumferentially around the piston as shown in FIGURE 3. The adhesive backing of the tape may be conductive or insulating. If the adhesive backing is conductive, the tape may be applied in overlapped horizontal layers and have adequate conductivity both vertically and horizontally. If the adhesive backing is insulating, the tape may be applied in overlapped vertical layers and have adequate vertical conductivity.

In the modification shown in FIGURE 4, the lead wires 46 may be stopped off with an insulating masking tape 50 which terminates at the corner 52 representing the juncture of the horizontal surface 38 of the groove opposite the land 14 and the vertical outer surface 40 of the piston as a further means of confining current flow to the lead tape surface within the ring groove itself. This more closely controls the distribution of metal to be deposited upon the bottom horizontal or land surface 14.

In the process of plating the land surface 14 with chromium, the vapor degreased piston 10 is supported, as described hereinabove, in a chromic acid plating bath 54. Before doing so, the land is preferably vapor blasted to produce an oxide-free surface. The piston is first electrically connected to the positive terminal of a suitable D.C. source, such for example as 6 volts, the lead tape electrode 32 being connected to the negative terminal by means of the lead wires 48. The land surface 14 is then given a conventional "reverse" etch at about 0.5-3 a.s.i. (72 to 432 a.s.f.) for one-half to several minutes. The electrical connections are then quickly reversed, preferably by a reversing switch, and the land surface 14 is chromium plated using the exposed surface of the lead tape 32 as the insoluble anode.

The composition of the chromium bath is not critical and current densities and temperatures of conventional values may be employed. The same is true when the land surface is to be plated with nickel, copper and other metals as mentioned hereinbefore. Satisfactory chromium plating of the land surfaces of cast iron diesel engine

pistons was accomplished with a temperature of 132° F. using a bath containing 36 oz./gal. of chromic acid with sufficient sulfuric acid to give a ratio of CrO<sub>3</sub> to H<sub>2</sub>SO<sub>4</sub> of 100 to 1. The current density must be varied in a conventional manner depending upon the temperature and the basis metal. Values of 0.5 to 3 a.s.i. (72 to 432 a.s.f.) may be used for copper, nickel and most steels. Lands of cast iron pistons were successfully plated by first striking for 1.5 to 2 minutes at 9 a.s.i. (1296 a.s.f.) and then continued deposition at 3 a.s.i. (432 a.s.i.). Steel pistons were successfully plated at the latter value without striking.

By the present invention, lands of new diesel pistons have been plated with 0.5 to 1.0 mil chromium wherein the coating of the deposited metal was sufficiently uniform over the entire land surface 14 to meet tolerances, thus eliminating the necessity of costly and difficult regrinding after plating. These pistons showed no appreciable wear on the plated lands after 1,000 hours test run.

It should be understood that the invention may also be employed to salvage worn pistons in which case the ring groove has been ground to give a true surface with a finish of 16 micro inch R.M.S. or better and chromium has been deposited up to a thickness of 6-12 mil which is not limiting. These heavier coatings may require regrinding to meet dimensional requirements, but even if they do such regrinding will be minimal since, by the present process, the thick chromium deposit is substantially uniform across the entire face of the land surface.

While a preferred embodiment of the invention has here been shown and described, skilled artisans may make minor variations without departing from the spirit of the invention and the scope of the appended claims. Thus, it should be understood that while it is the lands of pistons which are normally subject to wear and/or corrosion and therefore require plating, the invention is applicable to any metallic grooved member for the plating of any one or more surfaces of the groove which require a protective coating of metal.

I claim:

1. A process of electroplating a selective surface within a groove of a metallic structure comprised of affixing via insulating adhesion an insoluble deformable metallic member to the surfaces of the groove which are not to be plated, said member conforming to the configuration of the grooved surfaces to which it is affixed and having a portion within the groove opposing said selective surface to be plated, insulating all surfaces of said structure other than said selective surface and those covered by said insoluble metallic member and operatively connecting said member and structure to positive and negative poles respectively of a current source while subjecting said structure to a plating bath until a coating of metal of desired thickness is deposited on said selective surface.

2. A process of electroplating a selective surface within a groove of a metallic structure comprised of affixing insulating material to the member and to those surfaces of the groove which are not to be plated, adhesively affixing to a portion of the insulating material an insoluble deformable metallic tape so that it conforms to the contour of the surfaces covered and a portion of the tape is disposed within the groove in opposed position to the selective surface to be plated, and connecting the tape and structure to the positive and negative poles of a current source while subjecting the structure to a plating bath.

3. The process of claim 2 wherein the insulating material is deformable and affixed to the member by adhesion so that it conforms to the contour of the surfaces covered thereby.

4. The process of claim 2 and adhesively affixing to the outer face of the tape a strip of insulating material in such a position that the current from the tape to the selective surface is confined within the groove.

5. A process of chromium plating the land surface of the ring groove of a piston comprised of affixing an insulating material by adhesion to the surfaces of the piston other than the land surface, affixing to a portion of the material by adhesion a deformable lead tape so that it conforms to the surfaces covered and a portion of the tape is disposed within the groove in opposed position to the land surface, and connecting the tape and piston to the positive and negative poles of a current source while subjecting the piston to a chromium plating bath.

6. The process of claim 5 and affixing to the outer face of the tape by adhesion a second strip of insulation which terminates at the corner of the groove opposite

the land surface whereby the current from the tape to the selective surface is confined within the groove.

References Cited in the file of this patent

UNITED STATES PATENTS

|    |           |            |       |               |
|----|-----------|------------|-------|---------------|
| 5  | 1,335,176 | Merritt    | ----- | Mar. 30, 1920 |
|    | 1,798,391 | Wurth      | ----- | Mar. 31, 1931 |
|    | 1,809,872 | Solderberg | ----- | June 6, 1931  |
|    | 1,845,052 | Laukel     | ----- | Feb. 16, 1932 |
| 10 | 2,710,834 | Vrilakas   | ----- | June 14, 1955 |
|    | 2,859,157 | Curtiss    | ----- | Nov. 4, 1958  |

FOREIGN PATENTS

|         |               |       |               |
|---------|---------------|-------|---------------|
| 579,941 | Great Britain | ----- | Aug. 21, 1946 |
|---------|---------------|-------|---------------|